# EUROPEAN PATENT SPECIFICATION

(11) **EP 1 027 717 B1**
(45) Date of publication and mention of the grant of the patent: **08.09.2004**
(21) Application number: 98957250.8
(22) Date of filing: 26.10.1998
(51) Int. Cl.: H01J 29/18, H01J 9/22

(54) **CATHODOLUMINESCENT SCREEN WITH A COLUMNAR STRUCTURE, AND THE METHOD FOR ITS PREPARATION**
KATHODOLUMINESZENZSCHIRM MIT SÄULENFÖRMIGER STRUKTUR UND VERFAHREN ZUR HERSTELLUNG
ECRAN CATHODIQUE LUMINESCENT POSSEDANT UNE STRUCTURE EN COLONNES ET PROCEDE DE FABRICATION

(30) Priority: 27.10.1997 RU 97117737; 31.12.1997 RU 97122024
(43) Date of publication of application: 16.08.2000
(73) Proprietor: Crystalls and Technologies, Ltd., 117335 Moscow (RU)
(72) Inventor: GIVARGIZOV, Evgeny Invievich, Moscow, 117421 (RU); ZADOROZHNAYA, Ljudmila Alexandrovna, Moscow, 117331 (RU); STEPANOVA, Alla Nikolaevna, Moscow, 119270 (RU); SOSHHIN, Naum Petrovich, Fryazino, 141120 (RU); CHUBUN, Nikolai Nikolaevich, Fryazino, 141120 (RU); GIVARGIZOV, Mikhail Evgenievich, Moscow, 117133 (RU)
(74) Representative: Einsel, Martin
(86) International application number: PCT/RU1998/000347
(87) International publication number: WO 1999/022394

(56) References cited:
- EP-A- 0 481 465
- WO-A-94/18694
- WO-A-95/26037
- WO-A-97/19460
- US-A- 3 535 138
- US-A- 4 239 791
- US-A- 4 556 620
- US-A- 5 378 962
- US-A- 5 445 846
- PATENT ABSTRACTS OF JAPAN vol. 004, no. 133 (E-026), 18 September 1980 & JP 55 088249 A (TOSHIBA CORP), 3 July 1980

## Description

The present invention relates to the area of electronic materials and to microelectronics, including vacuum microelectronics, in particular to devices based on field emission, such as field-emission displays, vacuum fluorescent displays, cathodoluminescent lamps, etc. Particularly, the invention relates to a cathodoluminescent mosaic screen on a light-transparent substrate, said screen having light-emitting, light-guiding, dielectric and electro conductive light-absorbing components, the light-emitting components of the screen are implemented as light-guiding crystalline columns, one butt-end of the columns being fixed to an inner surface of the substrate. Further, the invention relates to a method for preparation of luminescent screens consisting of crystalline columns of luminescent material deposited on substrates.

The prior art luminescent screens are produced, as a rule, in the shape of crystalline films that are prepared, for example, by deposition from a vapour phase onto a smooth, for example, glass substrate.

For the deposition, techniques of evaporation of materials in vacuum, of sublimation, of chemical transport, of cathode sputtering, etc. are used.

In all the techniques, the nucleation of the crystalline luminescent materials (phosphors) occurs in a non-controlling manner, homogenously or heterogeneously, on a smooth structure-less substrate. At that case, the phosphors are usually a collection of tiny (micron and/or submicron) crystalline grains, usually isometric, approximately spherical shape superposed one onto another (Fig. 1). In such a system, the light generated in a crystalline grain (i.e., designated by a cross) is repeatedly scattered in the labyrinth of surrounding phosphor grains. This phenomenon deteriorates the resolution of the screen.

One more problem relates to the fact that in the film screen, consisting of the crystalline grains, not all the space is filled by the phosphor. This decreases the effectivity of the screen and deteriorates its thermo- and electro conductivity.

In addition, such screens have a bad adhesion to substrates because the approximately-spherical crystalline grains have only point contacts with the substrates.

In addition, when the luminescent screen is coated by a conductive light-reflective aluminium film, it is necessary to deposit an intermediate layer of a non-phosphor, thermally unstable material onto the aluminium film in order to ensure a good reflectivity of light from the film.

According to a suggestion made in EP 0 232 586 A2, single-crystalline (plate-like or epitaxial-layer) materials are used as phosphors. This improves reproducibility of characteristics of the screen and increases its effectivity (the ratio of the light energy to the energy expended for the light excitation). However, at such a case, the emitting light propagates along the plate (or along the expitaxial layer) of the phosphor; this deteriorates the resolution and the effectivity of the screen.

The EP 0 170 310 B1 supposes localized deposition of a phosphor from a diluted solution or suspension by spinning into holes, side walls of the holes being metallized in order to exclude penetration of the light into neighbour areas of the luminescent screen. However, at this case, contrast of the image is increased for only 50 %; in other words, scattering of the light along the luminescent screen is not excluded.

These drawbacks can be eliminated if the luminescent screen is made of columnar crystallites that have elongated shape whose elongation direction is approximately perpendicular to the plane of the screen. Such an idea is realized in the design described in EP 0 062 993 A1. At such a case the light excitated at columnar crystallites of the phosphor guides. However, the method for preparation of such screens by melt crystallization is not suitable for many practically-important cases, e.g., for thin (0.1 - 1 micrometer thickness) flat luminescent screens used in field-emission displays.

JP 55-088249 A proposes a screen with columnar crystals where an insert of non-luminous black material adjacent to the columnar crystals was placed. Such an insert is able to increase an image contrast of the columns that are directly adjacent to the insert, while other columns that are not adjacent (are not contacted) to the insert are not able to increase their contrast. In addition, JP 55 088249 A does not give a method for preparation of such a screen.

It is an object of the present invention to further improve the optical properties of the screen, for example contrast, resolution or effectiveness. It is another object of the invention to provide a method for the preparation of screens with improved optical properties.

The first object is solved by a screen with a columnar structure characterized in that the columns are surrounded by gaps, said gaps being coaxial to the columns, the columns being single-crystalline, the diameter-to-height ratio of the columns ranges from 1:1 to 1:100, a ratio of an area of the substrate, coated by the columns, to the total areas of the substrate ranging from 10:1 to 1:10 whereas the remaining part of the substrate and all the volume of the structure including the gaps is filled by an electro conductive non-light-emitting medium, said electro conductive non-light-emitting medium having a coefficient of light absorption in respect to the emitting light greater than 20 %.

The second object is solved by a method as discussed above wherein an intermediate substance forming a liquid phase at the crystallization temperature, other than the luminescent material, is firstly deposited on the substrate and, then, wherein the luminescent material is deposited in the form of single-crystalline columns by vapour deposition on the substrate, and wherein the volume of the structure between the single-crystalline columns is filled with an electro conductive non-light-emitting medium.

In this invention, a luminescent screen is proposed that consists of light-guide micro components, the light-guide properties being provided by a high quality of elongated single-crystalline grains.

When the microstructure of a screen has been already optimised, a next problem is its activation and co-activation. This problem is also solved by a preferred embodiment of this invention.

In addition, a protection of the phosphor against destruction has been also realized. At the same time, evolution of cathode-poisoning components from the luminescent screen is also eliminated in this case.

A cathodoluminescent mosaic screen on a light-transparent substrate that (screen) contains light-emitting, light-guiding, dielectric, and electro conductive light-absorbing components is proposed where the light-emitting components of the screen are implemented as light-guiding single-crystalline columns. Diameter-to-height ratio of the columns ranges from 1:1 to 1:100. One butt-end of the columns is fixed to an inner surface of the substrate. A ratio of an area of the substrate, coated by the columns, to the total area of the substrate ranges from 10:1 to 1:10. Remaining part of the substrate and all the volume of the structure is filled by an electro conductive non-light-emitting medium that has a coefficient of light-absorption in respect to the emitting light greater than 20 %. The surface of the columns is coated by a mirror reflecting metallic layer. The outer butt-ends of the columns are coated by a light-emitting luminescent layer. The thickness of the layer is smaller than the height of the columns for at least one order of magnitude. The luminescent layer can be epitaxial in respect to the columns.

A method for preparation of the luminescent screens is proposed in this invention, too. The method consists in vapour deposition of the luminescent material where an intermediate substance, that is other than the luminescent material and that forms a liquid phase at the crystallization temperature, is firstly deposited on the substrate. After that, the luminescent material is deposited on such a substrate. The thickness of the intermediate substance is more than 10 nanometres and is smaller than 1 micrometer. The liquid phase is formed at a contact interaction of the intermediate substance with the substrate.

The intermediate substance is formed by more than one chemical elements. At least one of the chemical elements is operating as an luminescent activator or co-activator. The activator or co-activator is introduced into the luminescent material by means of ion implantation.

A microrelief of inhomogenities in structure and/or chemical composition is created on the substrate, the inhomogenities being of regular character, in particular, of crystallographically-symmetric character.

The luminescent material is coated by a thin layer of a material that is transparent for electrons. In particular, diamond or diamond-like material serve as the transparent material.

An embodiment and details of the present invention are described below, by way of example only, with reference to the accompanying drawings, in which are:
- **Fig. 1**: a scheme of a standard cathodoluminescent screen that is formed by a film of approximately isometric crystalline grain.
- **Fig. 2**: a scheme of a cathodoluminescent screen formed by a film, that consists of columns approximately perpendicular to substrate.
- **Fig. 3**: a scheme of propagation of light beams in the film shown in Fig. 2.
- **Fig. 4**: a SEM micrograph of a cleavage cross-section of a continuous film consisting of the columns.
- **Fig. 5**: a scheme of the cathodoluminescent screen with columnar structure when it is bombarded by electrons. The shaded upper parts of the columns show a level to which the electrons penetrate and where the light is excited.
- **Fig. 6**: a scheme of the cathodoluminescent screen. The upper butt-ends of the screen are coated by a light-emitting luminescent layer.
- **Fig. 7**: a scheme of the cathodoluminescent screen formed of columns with gaps between them.
- **Fig.8**: a SEM micrograph of the film that consists of columns with gaps between them (top view). The mosaic structure of the screen is seen.
- **Fig. 9**: a scheme of the cathodoluminescent screen shown in Figs. 7 and 8. The gaps are filled with an electro conductive non-emitting medium.

An embodiment and good version for the realization of the invention is the cathodoluminescent screen with columnar structure, as it is proposed here, as shown in Figs. 2 to 4.

The electron beams from a flat cathode, as it is usually considered in field-emission displays, are incident on the screen and penetrate into a thin surface layer exciting light in the layer (Fig. 5). Another version, where the columnar-structure screen is coated by a light-emitting luminescent layer, is shown in Fig. 6.

These screens are featured by some advantages, especially in respect to low-voltage field-emission displays.
1. By a high light and energetic output that is caused by its design. Owing to the total internal reflection from the walls of the columns, a light-guide effect takes place: the light propagates preferentially along the columns, do not passing beyond columns and do not passing into neighbour columns.
2. By a low light scattering during the light propagation along the columns. This determines a high resolution of the design. It is equal to the number of the light-emitting components per a length unit.
3. By a high adhesion to the transparent substrate, to which the columns are fixed by their butt-ends, i.e., the light-emitting components contact to the substrate by a large area. This is especially important for diode-type field-emission displays where large gradients of the electric field are able to break screen particles of the substrate.

The advantages of the cathodoluminescent screen having the columnar structure are realized here by a proposed technique. The technique is based on chemical or physical vapour deposition, a participation of a liquid phase in the deposition process being of principal importance. An effectivity of the technique is illustrated in Fig. 4 where the columnar structure of the luminescent material cadmium sulphide is shown.

It is to underline the principal idea of the proposed design of the cathodoluminescent screen: the propagation direction of light in each columnar component is paraxial (parallel) to the direction of the primary electron beam, that excites the light (see Fig. 3), whereas in the known (standard) screens, formed by superposition of approximately-isometric grains, the light excited by the cathodoluminescence can propagate not only paraxially with the electron beam but also perpendicularly to it, or in any arbitrary direction in respect to the electron beam (see Fig. 1).

As the design of the columnar screen was realized and used in concrete electron devices, some of its not-evident advantages were found.
(a) Luminescence brightness of different grains (columns in this case) becomes more uniform. In the standard cathodoluminescent screens, the brightness of various grains differs significantly (up to 50 % at distances of 25-30 micrometers) due to differences in sizes of emitting grains; this deteriorates transfer and fixation of qualitative images.
(b) Electrical and heat power dissipation by the columnar phosphors increases significantly (5 to 10 times) in comparison with the standard cathodoluminescent screens.
(c) The "burning out" of the columnar screens at an unexpected switching off the electron beam scanning is practically eliminated. In the standard cathodoluminescent screens the power sufficient for irreversible burning out of the screens is usually 0.1 W/element (here the element is an image element, i.e., a pixel), whereas preliminary testings of the proposed columnar screen indicate to increase of the parameter up to 1 W/element (here the element is a column).
(d) The background image contrast at an illumination with intensive light sources (sun, electric lamp, etc) is increased. Standard cathodoluminescent screens have the contrast value ***k*** = *b*_{image}/*b* <5, where *b* is the brightness of background, *b*_{image} is the brightness of the pixel. Testings of the screens based on the proposed columnar phosphor show the values ***k*** > 10 to 20.

A significant electric charge, accumulated by standard screens, is not completely removed even by metallic (for example, aluminium) coatings 0.1-0.5 µm in thickness that are usually formed on the surface of the standard cathodoluminescent screens. This manifests itself in numerous discharges that disturb a stable work of electron devices. The columns are surrounded by gaps coaxial to the columns (see Figs. 7 to 9). The remainder of the substrate area and all other volume of the screen is filled by an electro conductive non-light-emitting medium that has the coefficient of light absorption in respect to the emitting light greater than 20 %.

It is to note that the above-mentioned advantages of the columnar screens manifest themselves both in experimental (10x10 mm) and consumer (25x25 or 75x75 mm) sizes of the screens. In other words, the unique parameters of the proposed structure do not depend on the sizes.

Changes of cross-sectional sizes of the light-emitting elements have been studied in respect to characteristics of the screens in general. At the cross-sectional size of the light-emitting elements of about 1 µm and at the pitch distance of about 2 µm a light-emitting structure containing more than 2.5x10⁷ cm⁻² light-emitting elements has been prepared. The parameters are superior in resolution respectively to all known screens. It has been also found that the columnar structures with pitches of 20 µm, at a total number of the columns of 2.5x10⁵, can have important applications as screens of electron-beam devices and of transducers.

In order to improve characteristics of cathodoluminescent screens, the gaps (a space) around the columns can be filled by an electro conductive light-absorbing medium. The procedure consists in a dipping of the columnar structure into a melt of suitable oxides and/or sulphides. Another approach consists in the impregnation of the columnar structure in low-melting point compounds. As such, not only oxides like B₂O₃ (melting point 450 °C), V₂O₅ (melting point 670 °C), CdO (826 °C), PbO₂ (290 °C), Bi₂O₃ (817 °C), but also sulphides SnS (882 °C), Sb₂S₃ (550 °C) were used. In addition, metallic eutectics like Cd-Bi-Pn-Sn (melting point 65 °C) and Pb-Sn were tested, too. All the mentioned compositions absorb the light in the spectral sub range of 420 to 760 nanometres, therefore it is possible, in the mosaic columnar structure, to increase significantly the contrast value owing to an increased absorption of the side emission of the columns and of an external light passing through the transparent substrate.

It was studied an influence of the electro conductive medium on the luminescent properties of the screen formed by the mosaic columnar structure. In the case of the filling of the gaps between the columns by the eutectic metallic phase Cd-Bi-Pn-Sn, the resistivity of the filling phase was 1 to 20 Ohm cm at the value of the optical absorption > 10⁵ cm⁻¹. At the ratio of the substrate area, coated by the columns, to the area of the filling medium of 5:1, the coefficient of light reflection from the front surface of the screen is 20 %, while a similar columnar structure, that was not filled by the electro conductive medium, reflects 45 to 60 % of incident light.

Relationships between the height of the columns and the height level of the light-absorbing phase was not studied. In some preliminary experiments, the relationship was 2:1. Even such a value provided a run-off of the electron current densities of 1 to 10 A/cm².

The columnar elements of the mosaic screens can have an additional coating by a metallic (Al or Ag) mirror transparent for electron beams with energies > 5 keV.

## Claims

1. A cathodoluminescent mosaic screen on a light-transparent substrate,
said screen having light-emitting, light-guiding, dielectric and electro conductive light-absorbing components,
the light-emitting components of the screen are implemented as light-guiding crystalline columns,
one butt-end of the columns being fixed to an inner surface of the substrate,
**characterized in that** the columns are surrounded by gaps,
said gaps being coaxial to the columns,
the columns being single-crystalline,
the diameter-to-height ratio of the columns ranges from 1:1 to 1:100,
a ratio of an area of the substrate, coated by the columns, to the total areas of the substrate ranging from 1:10, to 1,
whereas the remaining part of the substrate and all the volume of the structure including the gaps is filled by an electro conductive non-light-emitting medium,
said electro conductive non-light-emitting medium having a coefficient of light absorption in respect to the emitting light greater than 20 %.

2. The screen according to the claim 1 wherein the surface of the columns is coated by a mirror reflecting metallic layer.

3. The screen according to the claim 1 wherein outer butt-ends of the columns are coated by a light-emitting luminescent layer whose thickness is smaller than height of the columns for at least an order of magnitude.

4. The screen according to the claim 3 wherein the luminescent layer is epitaxial in respect to the columns.

5. A method for preparation of luminescent screens consisting of crystalline columns of luminescent material deposited on substrates,
wherein an intermediate substance forming a liquid phase at the crystallization temperature, other than the luminescent material, is firstly deposited on the substrate and, then,
wherein the luminescent material is deposited in the form of single-crystalline columns by vapour deposition on the substrate, and
wherein the volume of the structure between the single-crystalline columns is filled with an electro conductive non-light-emitting medium.

6. The method according to the claim 5 wherein the thickness of the intermediate substance layer is more than 10 nanometres and smaller than 1 micrometer.

7. The method according to the claim 5 wherein the liquid phase is formed at a contact interaction of the intermediate substance with the substrate.

8. The method according to any of claims 5 or 6 wherein the intermediate substance is formed by more than one chemical element.

9. The method according to the claim 8 wherein at least one of the chemical elements is operating as a luminescent activator or co-activator.

10. The method according to the claim 5 wherein a microrelief or inhomogenities in structure and/or in chemical composition is created on the substrate.

11. The method according to the claim 10 wherein the inhomogenities are of a regular character.

12. The method according to the claim 11 wherein the inhomogenities have crystallographically-symmetric character.

13. The method according to any of the claims 5 to 12 wherein the activator or co-activator is introduced into the luminescent material by means of ion implantation.

14. The method according to the claim 13 wherein the luminescent material is coated by a thin layer of a material transparent to electrons.

15. The method according to the claim 14 wherein diamond or a diamond-like material serve as the transparent material.

## Patentansprüche

1. Mosaikartiger Kathodolomineszensschirm auf einem lichtdurchlässigen Substrat,
welcher Schirm lichtabstrahlende, lichtführende, dielektrische und elektrisch leitende lichtabsorbierende Komponenten besitzt,
wobei die lichtabstrahlenden Komponenten des Schirms als lichtführende kristalline Säulen ausgebildet sind,
wobei ein stumpfes Ende der Säulen auf einer inneren Oberfläche des Substrates befestigt ist,
**dadurch gekennzeichnet,**
**dass** die Säulen von Lücken umgeben sind,
welche Lücken koaxial zu den Säulen sind,
wobei die Säulen einkristallin sind,
wobei das Verhältnis von Durchmesser zu Höhe der Säulen zwischen 1:1 und 1:100 liegt,
wobei ein Verhältnis einer mit den Säulen beschichteten Fläche des Substrates zu den Gesamtflächen des Substrates zwischen 1:10 und 1:1 liegt,
während der verbleibende Bereich des Substrates und das gesamte Volumen der Struktur einschließlich der Lücken durch ein elektrisch leitfähiges nicht lichtabstrahlendes Medium angefüllt ist,
welches elektrisch leitfähige, nicht lichtabstrahlende Medium einen Lichtabsorptionskoeffizienten bezüglich des abgestrahlten Lichts von mehr als 20 % besitzt.

2. Schirm nach Anspruch 1, in welchem die Oberfläche der Säulen mit einer spiegelnden, reflektierenden Metallschicht beschichtet ist.

3. Schirm nach Anspruch 1, in welchem äußere stumpfe Enden der Säulen mit einer lichtabstrahlenden lumineszenten Schicht beschichtet sind, deren Dicke um wenigstens eine Größenordnung kleiner als die Höhe der Säulen ist.

4. Schirm nach Anspruch 3, in welchem die lumineszente Schicht hinsichtlich der Säulen epitaxial ist.

5. Verfahren zum Vorbereiten von lumineszenten, aus kristallinen Säulen aus auf Substraten abgeschiedenen lumineszentem Material bestehenden Schirmen,
in welchem eine Zwischensubstanz eine flüssige Phase bei der Kristallisationstemperatur bildet, die nicht das lumineszente Material ist, und zuerst auf dem Substrat abgeschieden wird, dann
in welchem das lumineszente Material in der Form von einkristallinen Säulen durch Gasphasenabscheidung auf dem Substrat gebildet wird, und
in welchem das Volumen der Struktur zwischen den einkristallinen Säulen mit einem elektrisch leitfähigen, nicht lichtabstrahlenden Medium angefüllt wird.

6. Verfahren nach Anspruch 5, in welchem die Dicke der Zwischensubstanzschicht mehr als 10 nm und weniger als 1 µm beträgt.

7. Verfahren nach Anspruch 5, in welchem die flüssige Phase bei einer Kontaktreaktion der Zwischensubstanz mit dem Substrat ausgebildet wird.

8. Verfahren nach einem der Ansprüche 5 oder 6, in welchem die Zwischensubstanz von mehr als einem chemischen Element gebildet wird.

9. Verfahren nach Anspruch 8, in welchem eines der chemischen Elemente als Lumineszensaktivator oder -koaktivator wirkt.

10. Verfahren nach Anspruch 5, in welchem ein Mikrorelief oder Inhomogenitäten in der Struktur und / oder in der chemischen Zusammensetzung auf dem Substrat erzeugt werden.

11. Verfahren nach Anspruch 10, in welchem die Inhomogenitäten einen regelmäßigen Charakter besitzen.

12. Verfahren nach Anspruch 11, in welchem die Inhomogenitäten einen kritsallographisch symmetrischen Charakter besitzen.

13. Verfahren nach einem der Ansprüche 5 bis 12, in welchem der Aktivator oder Koaktivator in das lumineszente Material mittels einer Ionenimplantation eingeführt wird.

14. Verfahren nach Anspruch 13, in welchem das lumineszente Material mittels einer dünnen Schicht aus einem für Elektronen durchlässigen Material beschichtet wird.

15. Verfahren nach Anspruch 14, in welchem ein diamant- oder diamantähnliches Material als durchlässiges Material dient.

## Revendications

1. Ecran mosaïque cathodoluminescent sur un substrat transparent à la lumière, ledit écran ayant des composants émettant de la lumière, guidant la lumière, diélectriques et électro-conducteurs absorbant la lumière,
les composants émettant de la lumière de l'écran sont réalisés sous forme de colonnes cristallines guidant la lumière,
une culée des colonnes étant fixée à une surface interne du substrat,
**caractérisé en ce que** les colonnes sont entourées par des espacements,
lesdits espacements étant coaxiaux aux colonnes,
les colonnes étant monocristallines,
le rapport diamètre sur hauteur des colonnes varie de 1:1 à 1:100,
un rapport d'une aire du substrat, revêtu par les colonnes, sur les aires totales du substrat variant de 1:10 à 1,
tandis que la partie restante du substrat et tout le volume de la structure comprenant les espacements. est remplie par un milieu électro-conducteur n'émettant pas de la lumière,
ledit milieu électro-conducteur n'émettant pas de la lumière ayant un coefficient d'absorption de la lumière par rapport à la lumière d'émission supérieur à 20 %.

2. Ecran selon la revendication 1, dans lequel la surface des colonnes est revêtue par une couche métallique à réflexion miroir.

3. Ecran selon la revendication 1, dans lequel des culées externes des colonnes sont revêtues par une couche luminescente émettant de la lumière dont l'épaisseur est plus petite que la hauteur des colonnes d'au moins un ordre de grandeur.

4. Ecran selon la revendication 3, dans lequel la couche luminescente est épitaxiale par rapport aux colonnes.

5. Procédé de préparation d'écrans luminescents consistant en des colonnes cristallines de matière luminescente déposée sur des substrats,
dans lequel une substance intermédiaire formant une phase liquide à la température de cristallisation, autre que la matière luminescente, est tout d'abord déposée sur le substrat, puis
dans lequel la matière luminescente est déposée sous la forme de colonnes monocristallines par dépôt de vapeur sur le substrat, et
dans lequel le volume de la structure entre les colonnes monocristallines est rempli avec un milieu électro-conducteur n'émettant pas de la lumière.

6. Procédé selon la revendication 5, dans lequel l'épaisseur de la couche de substance intermédiaire est supérieure à 10 nanomètres et plus petite que 1 micromètre.

7. Procédé selon la revendication 5, dans lequel la phase liquide est formée à une interaction de contact de la substance intermédiaire avec le substrat.

8. Procédé selon l'une quelconque des revendications 5 ou 6, dans lequel la substance intermédiaire est formée par plus d'un élément chimique.

9. Procédé selon la revendication 8, dans lequel au moins l'un des éléments chimiques fonctionne comme un activateur ou co-activateur luminescent.

10. Procédé selon la revendication 5, dans lequel un microrelief ou des inhomogénéités en structure et/ou en composition chimique sont créés sur le substrat.

11. Procédé selon la revendication 10, dans lequel les inhomogénéités sont d'un caractère régulier.

12. Procédé selon la revendication 11, dans lequel les inhomogénéités ont un caractère cristallographiquement symétrique.

13. Procédé selon l'une quelconque des revendications 5 à 12, dans lequel l'activateur ou co-activateur est introduit dans la matière luminescente au moyen d'une implantation ionique.

14. Procédé selon la revendication 13, dans lequel la matière luminescente est revêtue par une fine couche d'une matière transparente aux électrons.

15. Procédé selon la revendication 14, dans lequel du diamant ou une matière de type diamant sert de matière transparente.
